

# UNITED STATES PATENT OFFICE.

JUDSON A. DE CEW, OF NEW YORK, N. Y., ASSIGNOR TO PROCESS ENGINEERS, INC., A CORPORATION OF NEW YORK.

## ROSIN SIZE SOLUTION.

1,382,346.

Specification of Letters Patent. Patented June 21, 1921.

No Drawing. Application filed April 10, 1919, Serial No. 289,126. Renewed April 13, 1921. Serial No. 461,150.

To all whom it may concern:

Be it known that I, JUDSON A. DE CEW, a subject of the King of Great Britain and native of the Dominion of Canada, residing 5 at 501 Fifth avenue, New York, N. Y., have invented certain new and useful Improvements in Rosin Size Solutions, of which the following is a specification.

While it is well known in the art that 10 paper may be made water repellent in the manufacturing process, by incorporating into the paper stock a solution of rosin soap and precipitating it upon the fibers by means of aluminum sulfate, with the formative of 15 acid resinate of aluminum, yet in spite of the most efficient methods of operation, there are some conditions in which the properties of rosin itself do not seem to be sufficient to meet the strains and destructive 20 mechanical conditions of the drying and calendering treatments.

The object of this invention is to so modify or alter the properties of rosin hydrates or complexes precipitated in the beating engine, 25 that they will be less liable to become dehydrated or otherwise destroyed during the drying process, and that the dried size will be more elastic and water repellent than before.

30 In order to accomplish this I incorporate into the size composition an oil or soap made from an oil which has special elastic and water repellent properties when dried, such as linseed, China wood or other so- 35 called varnish or drying oils.

The amount of these special oils or soaps that may be incorporated into the rosin size will depend upon the extent to which it is desired to modify the properties obtained 40 from rosin, but for purposes of overcoming the actions destructive to sizing on the paper machine, the quantity of these oils or soaps required may vary from 5 per cent. to 50 per cent. of the amount of rosin soap used.

45 When it is desired to make the rosin size particularly pliable, strong and water repellent, as much as 50 per cent. of the total size may consist of an oil soap compound made from a drying oil. Such sizes, when 50 precipitated with aluminum sulfate in the paper and dried on the paper machine undergo considerable oxidation; but, instead of the oxidation being destructive to

the sizing, as it is to rosin size alone, the properties of this blended material actually 55 develop and improve after oxidation.

The best sizing compound is produced when soap compounds made from drying oils are blended with a rosin soap containing a considerable amount of unsaponified 60 rosin.

One method of combining the properties of these two materials is to dissolve the unsaponified rosin in soap made from a drying oil, it being possible to dissolve together 65 equal quantities of rosin and such oil soap. Another method would be to dissolve a drying oil in a soap made from a drying oil and blend this with a rosin soap containing free rosin. 70

All of the sizing precipitates in which these oil soaps have been incorporated will be more fusible on the paper machine driers than those made from rosin size alone, and this property is one of the great advantages 75 arising from this composition, as it enables the sizing to re-melt when cracks are formed in drying, and as a result much more water-proof paper can be made.

Although this invention relates to improving rosin size, the real invention is the water-proofing quality of the precipitates of soaps made from a drying oil and in order to get certain ideal results regardless of expense, it may be desirable to use the oil soap 85 alone or emulsions of oil in the oil soap. 80

What I claim as my invention is:

1. A sizing composition having therein a 90 rosin soap, rosin, and a soap made from a drying oil.

2. A sizing composition having therein rosin and a soap made from a drying oil.

3. A sizing composition having therein rosin, rosin soap and a drying oil.

4. A sizing composition having therein 95 rosin soap and a drying oil.

5. A sizing composition having therein a drying oil, soap made from a drying oil, rosin and rosin soap.

6. A sizing composition having therein a 100 soap made from a drying oil containing an unsaponified oil.

In testimony whereof, I have signed my name to this specification, this seventh day of April 1919.

JUDSON A. DE CEW.